

Feb. 1, 1966

E. C. YACKEL ET AL

3,232,756

COLLOID TRANSFER PROCESS

Filed Aug. 20, 1962

FIG. 1



FIG. 2



FIG. 3



FIG. 4



EDWARD C. YACKEL  
HERBERT B. COWDEN

INVENTORS

BY *R. Frank Smith*  
*Henry E. Ryers*  
ATTORNEYS

1

3,232,756

**COLLOID TRANSFER PROCESS**

Edward C. Yackel and Herbert B. Cowden, Rochester, N.Y., assignors to Eastman Kodak Company, Rochester, N.Y., a corporation of New Jersey

Filed Aug. 20, 1962, Ser. No. 217,831

10 Claims. (Cl. 96—28)

This invention relates to a process in photography wherein an image in soft adhesive organic colloid is formed photographically and a discrete stratum of the image is transferred to a transparent receiving sheet to provide a reproduction of the subject, known as the colloid transfer process.

A typical colloid transfer process is described in the Yutzy et al. U.S. Patents 2,596,756, issued May 3, 1952 and 2,716,059, issued August 23, 1955. These patents disclose processes which embody the exposure to a subject of a substantially unhardened gelatino-silver-halide emulsion layer which may contain a gelatin tanning silver halide developing agent as well as a non-tanning silver halide developing agent. Upon activation of the exposed emulsion with an alkaline solution in the presence of the developing agent or agents, tanning development of the more exposed regions of the emulsion occurs corresponding to the highlights of the subject, although some development of the less exposed regions also takes place to provide visual density for the transferred image as explained in more detail in U.S. 2,716,059 above.

The developed emulsion is pressed into contact with an absorbent receiving sheet such as paper to cause the less exposed regions, and thus the less developed regions, of the emulsion to adhere to the receiving sheet. Subsequently, when the emulsion and receiving sheet are separated, a stratum of the less exposed regions of the emulsion remains on the sheet and appears as a positive silver image of the original subjects.

The alkaline solution which has been used for activation of the exposed emulsion layer has contained a gelatin softening agent to facilitate transfer of the less exposed portions of the emulsion to the receiving sheet. Urea and certain other gelatin softening agents have been used for this purpose.

In addition, sodium carbonate has been used as an alkaline component of the alkaline solution used for initiating development of the exposed emulsion.

It has been desired to have a transparent sheet for use as a receiving sheet in the colloid transfer process. For instance, such a transparent receiver sheet could be used in making copies for use with a projector which will project positive transparencies of an original onto a screen. In the past, such transparencies had to be prepared by inking or drawing the desired replica upon a matte surface and then projecting it.

One suggested solution to the problem of a transparent receiving sheet involves the use of colloidal silica dispersed in a binder such as cellulose acetate on a transparent support which might be cellulose triacetate or the like. However, when this type of transparent receiving sheet is used, the resulting image is not of satisfactory density, since the transferred gelatin does not adhere as well as to normally used paper receiving sheets.

We have found a method of making a transparent receiving sheet which not only provides a satisfactory surface for adhering the unhardened transferrable colloid image but which also results in an improved density of the image.

One object of this invention is to provide a simple photographic colloid transfer process for obtaining an image on a transparent support. Another object is to provide a transparent support which can be used in com-

2

mercially available colloid transfer processes without the use of additional steps. An additional object is to provide a coating for a transparent support which will be receptive to the adhesion of the transferrable colloid portion when used with the colloid transfer process. A still further object is to provide a coating for a transparent receiving sheet which results in an improved density of the image so that it can be used for projection purposes. Other objects will become apparent from the following description of our invention.

Our invention may be better understood by reference to the accompanying drawing wherein FIGURE 1 shows, in cross-sectional view, the appearance of a silver halide emulsion bearing support after exposure to a subject and development in the presence of a tanning developer.

FIGURE 2 shows, in enlarged cross-sectional view, the appearance of the transferred untanned emulsion image stratum in printing relation to the element of FIGURE 1.

FIGURE 3 shows, in enlarged cross-sectional view, a transparent receiving sheet which is identified as the transparent support shown in FIG. 2.

FIGURE 4 is a diagrammatic sectional view of typical apparatus, materials and methods used in our invention.

Our invention will now be described in greater detail with reference to the accompanying drawings.

In the preferred embodiment of our invention, the substantially unhardened light-sensitive, preferably pigmented, gelatino-silver-halide emulsion layer is exposed to an object and developed in the presence of a tanning developing agent incorporated into the emulsion layer. After exposure and development, the processed photographic element appears as shown in FIGURE 1 where, in enlarged cross-sectional view, layer 10 is a film, paper or other support to which is affixed the exposed and tanning developed silver halide emulsion layer 11 containing the silver and tanned gelatin image 12.

Next the moist element of FIG. 1 is placed in contact with the transparent receiving sheet 13 of FIG. 2 and by means of pressure and, if desired, the application of heat, the unexposed and untanned portion 16 of layer 11 is caused to adhere to the transparent support 13.

By rewetting the balance of image 16 on support 19 with the alkaline solution, additional transfers can be made.

FIGURE 4 illustrates a method of making prints by this process wherein the transparent sheet 13 is contacted with the tanned negative image in layer 11 and passed around hot roller 26 in order to increase the density of the image. The exposing light 24 at point 25 also improves the density of the image.

Since the coating of our invention renders transparent supports receptive to colloid transfer, various transparent supports may be used, such as glass or any of a number of transparent polymeric materials, including cellulose esters, polystyrene, polyethylene terephthalate, or the like. In our preferred embodiment, a transparent sheet of cellulose triacetate is used.

The polymeric sheeting is subbed with a suitable substrate commonly applied to film supports in order to obtain adhesion and then coated with a layer of suitable colloid containing a fogging agent for photosensitive silver halide, for example, thiourea, soluble sulfide, etc. In the event that a fogging agent is omitted from the receiving sheet, the image can be increased in density by exposing the receiving sheet to a photoflood lamp or to some other suitable source of radiation.

It will be appreciated that many of the transparent polymeric materials may require an additional surface treatment in order to obtain adherence of a subbing or coating composition. For instance, polyolefins, polyesters,

and the like, can be treated by electron bombardment, oxidation, chlorination, and the like, to improve the surface characteristics.

The colloid layer coated on the transparent support for reception of the image has been found to be critical, since many coatings will not result in a satisfactory image transfer, particularly if the material is not sufficiently absorbent. Moreover, if the colloid is too soluble in the activator solution, it tends to dissolve during contact with the exposed matrix with the resultant transfer of the colloid to the matrix. For instance, gelatin layers which are hardened with formaldehyde are usually not absorbent enough, while most gelatins are too soluble when coated unhardened. Moreover, bone and calf skin gelatins are too soft when coated unhardened and not absorbent when hardened by the usual methods. In addition, the sodium salts of ethyl cellulose phthalate or the sodium salt of the lactone of an interpolymer of vinyl acetate and maleic anhydride have not been found to be useful since they are too soluble.

We have found that pig gelatin can be used and also the ammonium salts of ethyl cellulose phthalate and the ammonium salts of the lactone of the interpolymer of vinyl acetate and maleic anhydride can be used. A further treatment may be used to prevent loss of ammonia from the ammonium ethyl cellulose phthalate salts and from the ammonia salt of the carboxy ester-lactones of an interpolymer of vinyl acetate and maleic anhydride which might cause these layers to become too insoluble so that insufficient water is absorbed and the materials lose their ability to accept a transfer. The coating can be heated such as by drying the coating at a high temperature. For instance, a temperature range of 220-240° F. may be used with ammonium ethyl cellulose phthalate. The surface may be treated with acid solutions, which convert the surface stratum of the coating to the impervious acid form of the colloid which seals the ammonia of the lower strata in the layer. The acid is not critical and dilute hydrochloric or acetic acid solutions as low as 2.5% concentration may be applied in an amount of about 3-4 ml./sq. ft. The concentration is not critical since the acid is volatilized when the coating is dried. The carboxy ester-lactone is a water-soluble salt of a carboxy ester-lactone of an interpolymer of maleic anhydride and vinyl acetate as described in U.S. Patent 3,007,901 of Louis M. Minsk, reacted with an aliphatic alcohol in such a ratio as to provide a polymer containing a carboxyl content between about 3.5 and 6 milliequivalents per gram of polymer and preferably between 4.5 and 5.5 milliequivalents per gram. The salt is then 25-98% neutralized with ammonia. A typical coating is disclosed in Sterman and Minsk U.S. patent application Serial No. 201,808.

The sodium or ammonium salt of a copolymer of ethyl acrylate and acrylic acid may also be used. In our preferred copolymer a 75% ethyl acrylate-25% acrylic acid proportion is used, but other proportions may be used. Conventional polymerization processes such as emulsion polymerization and the like may be used to prepare the copolymer.

The use of a matting agent such as silica of colloidal size or larger is not necessary to make these receiving materials work effectively, but it can be added to improve the latitude of the copying process with regard to exposure, activator temperature, and activator exhaustion. Another advantage obtained from the incorporation of matting agents is the ability to write with pencil or ball-point pen on the matted surfaces. Silica having a particle size ranging from about 3-30 microns in diameter are operative, but the preferred range is about 5-15 microns.

The thickness of the coated layers on these transparent receiving sheets may be from about 100 mg. of colloid per sq. ft. to one gram per sq. ft.

Our preferred thickness range is 250-400 mg. per sq. ft.

The following examples are intended to illustrate our invention but not to limit it in any way.

#### Example 1

5 A 5.5% solution of the ammonium salt of ethylcellulose phthalate containing 0.20% thiourea and having pH=7.6 was coated on a transparent cellulose ester film support (subbed side) at 7.3 g. solution per sq. ft., and dried to give a layer having 400 mg. colloid per sq. ft. When used as a receiver for the colloid transfer image, 10 dense black transfers were obtained which projected well on the Vu-Graph projector.

NOTE.—This sample of ethylcellulose phthalate contained 21.8% combined phthalyl and 1.6% free phthalic acid; its viscosity at 3% concentration in ethyl alcohol/isopropanol/n-butanol 70-20-10% was 4 cps. at 25° C.

#### Example 2

A solution like that used in Example 1 except that the thiourea was omitted and coated at the same coverage and set to a firm jelly by warming to about 60° C. In this condition, the coated layer was passed once through a 5% solution of acetic acid, and then dried as before. This material gave an excellent quality transfer when freshly made, and also after having been incubated for 14 days at 120° F., 35% R.H.

#### Example 3

30 A 4% solution of ammonium salt of a carboxy ester-lactone of an interpolymer of vinyl acetate and maleic anhydride in 1:1 acetone-water and containing 0.25% thiourea and 0.2% Syloid 404 (a silica dispersion) was coated at 10 g. per sq. ft. on the subbed side of a transparent cellulose ester film support and dried to give a layer having 400 mg. colloid per sq. ft. When dry, this sample was overcoated with 5% acetic acid applied at 3.5 g. per sq. ft., and again dried. This element used as a receiver with a colloid transfer matrix gave an excellent quality image of good density; after 28 35 days incubation at 120° F., 35% R.H., the material would still accept a high quality transfer.

#### Example 4

45 A 5% solution of high jelly strength pigskin gelatin containing 0.25% thiourea and 0.20% Syloid 404 was coated at 8 g. per sq. ft. on the subbed side of a transparent cellulose ester film support and dried to give a layer having 400 mg. gelatin per sq. ft. This element used as a receiver for a colloid transfer matrix gave a very high quality image of high density. Samples of this material incubated for 28 days at 120° F., 35% R.H. still accepted a high quality image of excellent density.

To facilitate drying, an alcohol-water solution can be utilized.

#### Example 5

55 Two coatings were made similar to the one described in Example 4 except Dimedone was added to the pig gelatin coating solution in sufficient quantities to give 2 and 5 mg. of Dimedone per sq. ft. After 3 months' aging, 60 the coatings containing the Dimedone gave a better quality transfer than the coatings without the Dimedone. Best results are obtained with coatings containing 0.5-10 mg. Dimedone per sq. ft.

Dimedone is described in U.S. Patent 2,944,899 as 65 5,5-dimethylcyclohexanone-1,3.

#### Example 6

70 A sample of the ammonium salt of a copolymer of 75% ethylacrylate and 25% acrylic acid containing 8.29% solids was diluted to 2.0% solids with water and coated on a transparent cellulose ester film support at a wet thickness of 0.005 inch. After drying, the coating was cured in an oven for 5 hours at 110° C. This element gave good transfers from colloid transfer matrices.

The alkali metal salts of the copolymer are operative and can be used without a stabilizing step.

The coating for the transparent support may also contain an agent which increases the density of the transferred image. For instance, a silver halide fogging agent (that is, a compound which renders silver halide developable in the absence of light), thiourea, thioacetamide, dithioxamide, and dithiobiuret, thiosemicarbazide, or a soluble sulfide may be used. A compound which retards the tanning of gelatin in the presence of fogged silver halide and the gelatin tanning agent may also be incorporated in the coating, for example, sodium formaldehyde bisulfite, sodium formaldehydesulfonate, 2,4-dihydroxybenzoic acid, sodium benzene sulfinate, borophosphate, aminomethanesulfuric acid, or borax.

It will be appreciated that the coatings may be surface applied or that the sheet can be surface coated or coated using any of the known coating methods, such as hopper coating, wick, kiss roll, knife, and the like.

The invention has been described in detail with particular reference to preferred embodiments thereof, but it will be understood that variations and modifications can be effected within the spirit and scope of the invention as described hereinabove and defined in the appended claims.

We claim:

1. In a process of photographic reproduction which comprises forming by exposure to a two-tone subject and development in a light-sensitive, substantially unhardened, organic colloid-silver halide emulsion layer, a hardened 30 colloid image and leaving substantially unhardened colloid in the remaining area of said layer, said unhardened layer being not harder than a gelatin layer containing 0.7 gram of formaldehyde per pound of gelatin freshly coated, the step of pressing the emulsion layer while said emulsion is moist against a nonfibrous, transparent polymeric sheet having thereon a non-light-sensitive coating selected from the class consisting of pig gelatin, the ammonium salt of ethylcellulosephthalate, the ammonium salt of a carboxy ester-lactone of an interpolymer 35 of maleic anhydride and vinyl acetate and the alkali metal and ammonium salts of a copolymer of ethylacrylate and acrylic acid, to cause only said unhardened colloid portion of said layer to adhere to said sheet, and separating said sheet and said emulsion layer to transfer only a

45 NORMAN G. TORCHIN, Primary Examiner.

stratum of the unhardened colloid portion of said layer to said sheet.

2. The process of claim 1 in which the coating on the transparent support is pig gelatin.

3. The process of claim 1 in which the coating on the transparent support is the ammonium salt of ethylcellulosephthalate.

4. The process of claim 1 in which the coating on the transparent support is the ammonium salt of a carboxy ester-lactone of an interpolymer of maleic anhydride and vinyl acetate.

5. The process of claim 1 in which the coating on the transparent support is an alkali metal salt of a copolymer of ethylacrylate and acrylic acid.

6. The process of claim 1 in which the coating on the transparent support is the ammonium salt of a copolymer of ethylacrylate and acrylic acid.

7. The process of claim 1 in which the coating on the transparent support contains 0.5-1.0 milligram per square foot of 5,5-dimethylcyclohexanone-1,3.

8. The process of claim 1 in which the coating on the transparent support contains a matting agent.

9. The process of claim 1 in which the coating on the transparent support contains a fogging agent.

10. The process of claim 1 in which the coating on the transparent support contains silica and thiourea.

#### References Cited by the Examiner

#### UNITED STATES PATENTS

|           |         |                     |       |          |
|-----------|---------|---------------------|-------|----------|
| 2,576,921 | 12/1951 | Buscher             | ----- | 117-164  |
| 2,596,756 | 5/1952  | Yutzy et al.        | ----- | 96-28    |
| 2,858,238 | 10/1958 | Brown               | ----- | 117-164  |
| 2,865,745 | 12/1958 | Chan et al.         | ----- | 96-28    |
| 2,944,899 | 7/1960  | Damschrader et al.  | ----- | 96-95    |
| 2,992,213 | 7/1961  | Gates et al.        | ----- | 96-87    |
| 3,043,688 | 7/1962  | Weyerts et al.      | ----- | 96-28    |
| 3,060,023 | 10/1962 | Burg et al.         | ----- | 96-87    |
| 3,062,674 | 11/1962 | Houck et al.        | ----- | 96-87    |
| 3,072,482 | 1/1963  | Beeber et al.       | ----- | 96-87    |
| 3,080,230 | 3/1963  | Haydn et al.        | ----- | 96-28    |
| 3,108,995 | 10/1963 | Tourtellotte et al. | ----- | 96-111 X |